

## UNITED STATES PATENT OFFICE

2,476,418

## DESILICONIZATION OF FERROPHOSPHORUS

Bethune G. Klugh, Anniston, Ala., assignor to  
Monsanto Chemical Company, St. Louis, Mo.,  
a corporation of Delaware

No Drawing. Application April 29, 1947,  
Serial No. 744,797

9 Claims. (Cl. 75—132)

1

The present invention relates to ferrophosphorus of substantially reduced silicon content and to an improved method of manufacturing same. More particularly, the invention is concerned with the production of substantially silicon-free ferrophosphorus which is particularly suitable for use in the steel industry.

Ferrophosphorus is used in the production of steel products requiring rephosphorization, such as "rimmed steel." This specific character of steel is essential in a number of important finished products, particularly thin steel sheets which require a small phosphorus content for effecting the required stiffness. "Rimmed steel" differs in character and method of production from that general type called "killed steel," the primary difference being that the "rimmed steel" must have the ingots cast without a deoxidizing or "killing" agent of the ferro-silicon class. This practice in regard to "rimmed steel" has been definitely established by substantially all of the experts in the art and consequently they demand a ferrophosphorus with as low silicon content as possible.

There are certain types of steels which can use a high silicon ferrophosphorus for their purpose, but low silicon ferrophosphorus can be used equally as well and hence the steel industry prefers a product of sufficiently low silicon content for "rimmed steel" so that a single stock of this alloy will be adapted to all its uses.

Commercially, ferrophosphorus is produced as a by-product of the thermal method of manufacturing elemental phosphorus or phosphoric acid which involves heating phosphate rock, a silicious flux and a carbonaceous reducing agent in an electric or blast furnace. By properly adjusting the furnace and burden conditions, it is possible to directly produce ferrophosphorus having a low content of silicon, but this method of operation is inconsistent with low maintenance, high phosphorus recovery and readily controlled furnace operation. Consequently, it is a more economical practice to produce ferrophosphorus having a relatively high silicon content and then effect a separation of the silicon by a subsequent treatment.

It has already been proposed to mix molten ferrophosphorus rich in silicon and obtained in the volatilization of phosphorus with fresh quantities of raw phosphate, preferably tricalcium phosphate, and then fuse the resulting mixture in a non-oxidizing atmosphere, whereby the phosphate is reduced by the silicon contained in the ferrophosphorus. The silica formed as a result of this reaction combines with the lime liberated from the phosphate to produce a silicate

2

slag and the phosphorus liberated by the reduction is partially taken up by the ferrophosphorus, thereby increasing the phosphorus concentration in the alloy. The elemental phosphorus which does not combine with the alloy escapes and is condensed or burnt to form phosphoric acid in the conventional manner.

The above method has achieved some measure of success, but it has been by no means entirely satisfactory, principally because of the difficulty of bringing about the following reaction without effecting substantial depophosphorization of the ferrophosphorus:

15 (1)



For example, a competing reaction which may occur in the high temperature contact of phosphate material with ferrophosphorus is that of the accepted form in the elimination of phosphorus in steel manufacture. This reaction occurs in two steps as follows:

25 (2)



Net reaction of (2) and (3):

30 (4)



It is to be noted that in the above phosphorus removal reactions the reactant material is not tricalcium phosphate, but  $\text{FeO}$  and  $\text{CaO}$ . However, both of these oxides occur in effective proportions in the phosphate materials available and hence reaction 4 must be avoided if satisfactory silicon removal is to be obtained without substantial depophosphorization of the ferrophosphorus.

Moreover, it can be demonstrated by thermal calculations that reaction 4 is exothermic to the degree of 3334 P. C. U. per pound of phosphorus involved as compared with 540 P. C. U. in reaction 1 and hence it is obvious that reaction 4 will take effect far ahead of reaction 1 if conditions favorable therefor exist.

50 Thus, it is evident that while the undesired reaction, that is, reaction 4 may not seriously interfere with the removal of silicon from ferrophosphorus, it has the very undesirable effect of reducing its phosphorus content and of increasing its iron content.

Another serious disadvantage of removing silicon from ferrophosphorus by means of tricalcium

phosphate flows from the fact that ferrophosphorus has a higher density than the phosphate material and consequently it separates from the latter before the reaction goes to completion. This difficulty arises not only when both materials, ferrophosphorus and phosphate material, are mixed together and heated up to the reaction temperature from the cold state but also when the reaction is carried out by contacting molten ferrophosphorus with cold phosphate material. As a result of this difficulty, ferrophosphorus having a variable silicon content is produced which is objectionable for obvious reasons.

The primary object of the present invention is, therefore, to provide a process of desilicizing ferrophosphorus in which the above difficulties and disadvantages are either completely eliminated or substantially reduced.

Another object of the invention is to provide an economical and effective method of removing silicon from ferrophosphorus without impairing the original desirable characteristics of the alloy.

An additional object is to provide a commercially feasible method of desilicizing ferrophosphorus while maintaining or increasing its phosphorus content.

A further object is to provide a process of desilicizing ferrophosphorus in which the desired reaction between the silicon of ferrophosphorus and tricalcium phosphate takes place to the substantial exclusion of the competing reaction hereinbefore described.

A still further object is to provide a low silicon ferrophosphorus which is eminently suitable for use in the steel industry.

Other objects and advantages will be apparent to those skilled in the art as the description proceeds.

In accordance with the present invention, tricalcium phosphate, phosphate rock or equivalent phosphate material is preheated to a temperature of at least 2500° F. and then contacted in a suitable furnace with silicon-containing ferrophosphorus, preferably in the molten condition, to form a silicate slag and ferrophosphorus of increased phosphorus content and substantially reduced silicon content, whereupon these products are successively tapped from the furnace in the conventional manner.

As indicated in the preceding paragraph, it is preferred to employ ferrophosphorus in the molten condition as it can be handled and treated in this condition with greater facility. However, it is within the scope of the present invention to employ the alloy in the cold state. In charging the cold alloy into the furnace, it is essential to successful operation that the phosphate reacting material be preheated to a temperature sufficient to combine the CaO, FeO and SiO<sub>2</sub> content thereof into silicates; that there be ample fusion of the phosphate material; and that the fused phosphate material be of sufficient depth to immerse the charged alloy. In practice, it is preferred to charge the cold alloy in the finely divided state and in small increments in order that its submergence in the fused reactant be assured.

The preheating step is a critical feature of the invention and should be carried out at a temperature of at least 2500° F. as a temperature of this magnitude is required to complete the reaction of SiO<sub>2</sub> and the free CaO and Fe<sub>2</sub>O<sub>3</sub> of the phosphate material into silicates. This step achieves two important functions which result in the production of a desilicized product having an in-

creased phosphorus content instead of a similar product of decreased phosphorus content. First of all, by bringing about the formation of the above stable silicates, it prevents reaction 4 from taking place when the phosphate material is contacted with the ferrophosphorus. In addition, it ensures complete or substantially complete reaction between the silicon content of the ferrophosphorus and the phosphate material as the latter has no cold spots to which the ferrophosphorus can penetrate and be cooled to a point below the desilicization temperature.

The desilicization of ferrophosphorus is effected by reacting its silicon content with tricalcium phosphate in at least the theoretical proportions defined in reaction 1, but in order to ensure maximum silicon removal, it is preferred to employ an excess of phosphate material. In fact, in view of the severe corrosion problems involved, it is desirable to use an excess of phosphate material which is large enough to function as a liner for the furnace or reactor as the life of the latter is thereby greatly increased.

In carrying out the desilicization reaction, the phosphate and ferrophosphorus should be brought together under conditions ensuring uniformity of heating and the maximum possible contact between these materials. This can be best accomplished by the use of a reverberatory furnace, but it is to be clearly understood that the invention is not restricted thereto.

The invention is illustrated but not limited by the following examples:

#### Example I

150 lbs. of ferrophosphorus containing 3.05% by weight of silicon and 20.68% by weight of phosphorus was heated to a temperature of from 2710° F. to 2860° F. and tapped into a long narrow reverberatory furnace containing 160 lbs. of phosphate concentrates which were preheated to a temperature of 2710° F. and arranged in the form of a trough for the molten metal. After tapping, the reactants were heated for 1 hour and 55 minutes at a temperature of from 2660° F. and 2800° F. by means of a natural gas-hot air blast, and the products obtained consisted of ferrophosphorus containing 25.05% by weight of ferrophosphorus and 0.10% by weight of silicon and a calcium silicate slag.

In this example, it will be noted that reaction 1 prevailed over reaction 4 as the phosphorus content of the original alloy was increased and its silicon content was substantially decreased.

#### Example II

81 lbs. of phosphate material was introduced into a circular reverberatory furnace in such a manner as to provide therein an inverted conical container space. 25 lbs. of finely divided ferrophosphorus was then charged into the furnace and arranged in the container space in the form of a conical pile of the alloy. After charging the furnace in the above manner, the reactants were heated by means of a gas flame in accordance with the following schedule:

| TIME  | TEMPERATURE IN FURNACE |
|-------|------------------------|
| 11:11 | Started Heat           |
| 1:15  | 2100° F.               |
| 2:21  | 2340° F.               |
| 2:43  | 2500° F.               |
| 4:00  | 2600° F.               |
| 6:00  | 2570° F.               |

The results obtained by the above heating operation are indicated below:

|                                                  | Per Cent<br>P  | Per Cent<br>Si |
|--------------------------------------------------|----------------|----------------|
| Ferrophosphorus Charged To Reverberatory Furnace | 22.95<br>19.94 | 2.74<br>0.10   |
| Ferrophosphorus Product of Treatment             |                |                |

This example demonstrates that when ferrophosphorus and the phosphate material are brought up to reaction temperature from the cold state, reaction 4 occurs as well as reaction 1, since substantial dephosphorization accompanies desiliconization.

*Example III*

150 lbs. of ferrophosphorus was melted in an electric furnace and tapped at a temperature of from 2900° F. to 2930° F. into a narrow elongated reverberatory furnace containing phosphate concentrates which were preheated to 2500° F. and arranged in the form of a trough for the molten metal. Upon completing the tapping operation, the molten metal in contact with the concentrates was heated to a temperature of from 2590° F. to 2770° F. for 1 hour and 58 minutes by means of a natural gas-hot air blast to yield a calcium silicate slag and ferrophosphorus of increased phosphorus content and relatively low silicon content. The extent of the desiliconization and phosphorization of the ferrophosphorus is indicated by the following data:

|                                                  | Per cent<br>P  | Per cent<br>Si |
|--------------------------------------------------|----------------|----------------|
| Ferrophosphorus Charged To Reverberatory Furnace | 20.55<br>23.52 | 4.26<br>0.10   |
| Ferrophosphorus Product of Treatment             |                |                |

The use of a temperature of at least 2500° F. is critical insofar as the preheating step is concerned as all efforts to effect this operation at a lower temperature have resulted in failure. For example, an attempt was made to desiliconize ferrophosphorus by contacting phosphate materials preheated to 2470° F. with molten ferrophosphorus (2820° F.), but as indicated by the following results, the attempt was completely unsuccessful.

|                                                  | Per cent<br>P  | Per cent<br>Si |
|--------------------------------------------------|----------------|----------------|
| Ferrophosphorus Charged To Reverberatory Furnace | 21.17<br>21.21 | 3.80<br>3.22   |
| Ferrophosphorus Product of Treatment             |                |                |

The method of desiliconizing ferrophosphorus hereinbefore described yields a product of greatly increased commercial importance over the original material. Thus, the desiliconized product has a higher content of phosphorus than the original material and hence less of it is required to supply the same quantity of phosphorus. Moreover, since it contains less than 1% by weight of silicon, it is particularly suitable for use by the steel industry as now a single stock of this alloy will be adapted to all its uses, including the production of "rimmed steel."

The various operating conditions of the present process of desiliconizing ferrophosphorus will now be summarized.

In the desiliconization reaction, it is essential that the phosphate material be preheated to a

temperature of at least 2500° F., and preferably above that temperature, to produce stable silicates from the SiO<sub>2</sub> and the free CaO and FeO contained in the phosphate material. This has the effect of preventing reaction 4 from taking place when the phosphate material is contacted with molten ferrophosphorus; it also facilitates substantially complete desiliconization by eliminating cold spots within the phosphate material which reduce the temperature of the higher gravity ferrophosphorus to a point below the desiliconization reaction temperature.

In addition, it is essential that there be sufficient molten phosphate material to cover the ferrophosphorus introduced for contact and reaction therewith. The ferrophosphorus should also have adequate time and contact with the phosphate material in order to complete the reaction for removal of all or substantially all of the silicon in the metal.

The ferrophosphorus is preferably in the molten condition when brought into contact with the phosphate material, but as indicated earlier herein it may be employed in the cold state provided the alloy is added to the fused phosphate material in the finely divided state and in such amounts and under such conditions as to be immersed in the fused material or at least be supplied with a film thereof. These requirements must be met in order to achieve successful operation as if any unfused alloy is exposed to combustion or oxidizing gases, the formation of FeO takes place which accelerates reaction 4 and thereby results in dephosphorization of the alloy.

In operating in accordance with the preferred procedure, it is desirable that the ferrophosphorus be of high fusion temperature, that is, at least as high as 2540° F. and under no circumstances, whether before or after supplemental heating, should the temperature of the ferrophosphorus or the phosphate material be low enough to reduce the resultant temperature below 2400° F. and preferably not below 2500° F.

Thus, if the phosphate material is initially preheated to a temperature of at least 2500° F., the desiliconization reaction may be carried out at a temperature of from 2400° F. up to 3300° F. or higher temperature, starting with either cold or molten ferrophosphorus.

As hereinbefore indicated, the phosphate material may be used in substantially the theoretical proportions required by Equation 1, but it is desirable to use an excess in order to ensure substantially complete removal of silicon. In fact, in view of the corrosion problems involved, it is preferable to use an excess of phosphate which is large enough to provide a liner for the furnace or reactor. The thickness of the liner will vary widely with the operation conditions, but in general, a liner thickness of about 12 inches has been found to be satisfactory. However, where sufficiently resistant equipment is available, no advantage from the standpoint of desiliconization is achieved by using greater than 8% excess of phosphate material.

The time required for completion of treatment of a given quantity of ferrophosphorus is largely governed by the reaction temperature and the relative area of contact of the molten metal and the molten phosphate material entering the reaction. Under the conditions prevailing in the present process where the previously heated phosphate material in the furnace is largely in fluid form, the molten alloy entering the furnace will have interfacial reactant contact completely en-

veloping the metal section of the bath and hence the reaction will proceed at a high rate. In fact, under the preferred operating conditions, where the reaction is carried out in a reverberatory furnace with maximum surface contact and at relatively high temperature that is, above 2600° F., the desiliconization reaction will take place within a period of several minutes.

With reference to the apparatus, it is desirable that the phosphate materials function as the bottom and sidewalls of the furnace or reactor in the desiliconization reaction, and the charging means for the phosphate materials must be of such arrangement that the portion consumed in the smelting operation will be automatically replaced. This requirement may be met by the use of a large excess of phosphate material in the initial furnace charge or by providing for gravity filling from storage into the furnace.

The furnace hearth formed by the phosphate reactant material within the furnace proper must provide for a relatively narrow and shallow receptacle space within which the molten ferrophosphorus will flow, so that the maximum obtainable area of contact of the metal and reactant phosphate in solid, pasty or liquid state is available for the required reaction.

The entire area in which the reaction proceeds must be uniformly heated to a temperature within the range of from 2400° F. to 3300° F. or a higher temperature so as to avoid inactive or dormant "pockets." This is important for the following reasons:

If there is any small section in which the temperature is below that required for the desiliconization reaction, the alloy will not be desiliconized to the desired degree.

If a portion of the reactant phosphate material does not reach the temperature required to complete the reaction of  $SiO_2$  and the free  $CaO$  and  $FeO$  content thereof into stable silicates, they will function according to reaction 4 which produces dephosphorization and impairs the value of the product.

Moreover lack of uniformity of heating of the phosphate material in the hearth sections retards the progressive stages of the desiliconization reactions of the whole charge, thus degrading the product and/or extending the cycle period.

The mechanism of the desiliconization reaction involves interfacial film reactions of the alloy and of both the liquid phosphate material on top and the pasty state at the bottom of the furnace.

The normal initial bisilicate reaction product is quite fluid at the temperatures prevailing in the present desiliconization process and it will tend to flow, thus producing the desired agitation of the reacting mass. It is desirable, however, to supplement this action by blowing the combustion gases in a tangential direction to the bath surface in order to effect the greatest possible movement.

The above requirements are provided in a reverberatory type of furnace, particularly one of circular arrangement. This form provides the greatest attainable uniformity of heat transfer conditions from gas flames. Thus, the phosphate material is charged peripherally around the side wall and in the center of the furnace, thereby producing a trough receptacle for the melting and liquid phase reactions. The phosphate filling effects the replacement of consumed reactant, and in addition functions throughout as the container wall and bottom for the liquid

material during the course of the conversion. Although a reverberatory type of furnace is preferred for use in the present desiliconization process, any other suitable furnace, including an electric furnace, may be employed which meets the above requirements as to uniformity of heat conditions and efficient surface contact between the reactants.

The expression "phosphate material" as used in the specification and claims is intended to cover tricalcium phosphate, raw phosphate rock, phosphate rock concentrates, phosphate sinter and mixtures thereof or equivalent materials.

While I have described above certain specific forms of my invention, it will be appreciated that it is susceptible to various changes and modifications without departing from the spirit thereof.

I claim:

1. The process which comprises contacting phosphate material preheated to a temperature of at least 2500° F. with ferrophosphorus rich in silicon and thereby forming a silicate slag and ferrophosphorus of relatively low silicon content.

2. The process which comprises contacting phosphate material preheated to at least 2500° F., with molten ferrophosphorus rich in silicon and thereby forming a silicate slag and ferrophosphorus of relatively low silicon content, said preheated phosphate material and said ferrophosphorus having a temperature of sufficient magnitude to maintain the resultant reaction temperature at a value of at least 2400° F.

3. The process which comprises contacting phosphate material preheated to at least 2500° F., with molten ferrophosphorus rich in silicon to form a silicate slag and ferrophosphorus of increased phosphorus content and substantially decreased silicon content, said phosphate material being employed in substantially the theoretical proportions required to oxidize the silicon content of said ferrophosphorus rich in silicon.

4. The process which comprises contacting phosphate material preheated to at least 2500° F., with molten ferrophosphorus rich in silicon to form a silicate slag and ferrophosphorus of increased phosphorus content and substantially decreased silicon content, said phosphate material being employed in an amount not exceeding about 8% excess of the theoretical proportion required to oxidize the silicon content of said ferrophosphorus rich in silicon.

5. The process which comprises contacting in a reverberatory type furnace phosphate material preheated to a temperature of at least 2500° F., with molten ferrophosphorus rich in silicon to form a silicate slag and ferrophosphorus of increased phosphorus content and substantially decreased silicon content, and thereupon successively tapping said slag and said alloy product from said furnace.

6. The process which comprises tapping molten ferrophosphorus rich in silicon onto phosphate material preheated to a temperature of at least 2500° F. and then maintaining the reactants at a temperature of at least 2400° F. until substantially complete desiliconization has taken place.

7. The process which comprises tapping molten ferrophosphorus rich in silicon onto phosphate material preheated to a temperature of at least 2500° F. and then maintaining the reactants at a temperature of at least 2400° F. by means of a gas flame until substantially complete desiliconization has taken place.

8. The process which comprises tapping molten

ferrophosphorus rich in silicon into a reverberatory type furnace lined with phosphate material which has been preheated to a temperature of at least 2500° F. and then heating the reactants to a temperature above 2600° F. to yield a silicate slag and ferrophosphorus of increased phosphorus content and substantially decreased silicon content.

9. The process which comprises tapping molten ferrophosphorus rich in silicon into a reverberatory type furnace lined with at least partially fused phosphate material and then heating the reactant materials to a temperature of at least 2400° F. to form a silicate slag and ferrophosphorus of increased phosphorus content and substantially decreased silicon content, said partially fused phosphate material being employed in

an amount sufficient to provide said tapped ferrophosphorus with at least a thin coating of said phosphate material.

BETHUNE G. KLUGH.

#### REFERENCES CITED

The following references are of record in the file of this patent:

#### UNITED STATES PATENTS

|    |           |       |               |
|----|-----------|-------|---------------|
| 10 | Number    | Name  | Date          |
|    | 2,430,671 | Feild | Nov. 11, 1947 |

#### FOREIGN PATENTS

|    |         |               |               |
|----|---------|---------------|---------------|
| 15 | Number  | Country       | Date          |
|    | 355,610 | Great Britain | Aug. 27, 1931 |